

1

3,796,579

**MULTIPLE-SPEED PHOTOGRAPHIC EMULSION  
CONTAINING AN ORGANIC COMPOUND OXI-  
DIZABLE TO A SPECTRAL-SENSITIZING  
DYE**

Leslie G. S. Brooker, deceased, late of Rochester, N.Y., by Lincoln Rochester Trust Company, executor, and Paul B. Gilman, Jr., Rochester, N.Y., assignors to Eastman Kodak Company, Rochester, N.Y.

No Drawing. Filed Apr. 10, 1972, Ser. No. 242,737

Int. Cl. G03c 1/02

U.S. Cl. 96—94 R

16 Claims

**ABSTRACT OF THE DISCLOSURE**

A multiple-speed photographic emulsion is provided by incorporating a colorless dye precursor in a photographic silver halide emulsion. After exposure, the emulsion is developed and a normal photographic image is obtained. During the course of development, the dye precursor is converted into an active spectral sensitizing dye in the areas of exposure. If higher photographic speed is desired, the element is then uniformly reexposed to radiation corresponding to the sensitivity of the spectral sensitizing dye and development is continued to obtain an amplified image corresponding to a relatively higher speed.

This invention relates to photography and more particularly to a novel multiple-speed photographic emulsion.

Normally, photographic emulsions have fixed or limited exposure latitude depending on the nature of the photographic emulsion, the type of energy to which it is exposed or the manner in which it is processed.

A typical black-and-white photographic emulsion has an exposure latitude of about two stops (a factor of 4). Such film must, therefore, be correctly exposed. Any miscalculation in presetting the camera controls will result in either under- or over-exposure of the film. A drastic miscalculation in exposure can result in unusable negatives.

Photographic materials with extended exposure latitude have been known. Such materials comprise multiple-layer coating with color couplers which are incorporated in the various speed silver halide emulsions. They are printed through selected complimentary filters. These filters make visible the image of a given color layer so that the layer which has received the proper exposure may be selected for printing. Such elements are disclosed, for example, in U.S. Pat. 3,450,530.

Other techniques have been described to amplify the initial response of a developing grain, such as by using the iodide ion released during development of a multilayer film to trigger development of internally fogged grains in another layer. This technique is described in Luckey et al. U.S. Pat. 2,996,382.

Although prior-art image-amplification techniques of the type indicated have offered a number of advantages, they have had certain drawbacks, particularly in the expense and difficulty of manufacture of the multiple-layer elements.

Accordingly, it is an object of this invention to provide novel multiple-speed photographic materials. Another object is to provide a novel photographic emulsion containing an incorporated sensitizing dye precursor. Still another object is to provide a method for amplifying photographic images and thereby increasing the speed of the photographic element. Another object is to provide a photographic element which can vary considerably in speed depending on whether or not the element is exposed a second time during or after the development step. It is still a further object of this invention to provide a method by which the oxidation products of photographic develop-

2

ment convert a colorless dye precursor into an active spectral sensitizer in an imagewise pattern which will result in photographic amplification when development takes place under minus blue light. Other objects will be apparent from the following specification and the appended claims.

These and other objects are obtained by our novel photographic emulsions, elements and methods of processing which provide for the amplification of the image of a photographic, spectrally unsensitized silver halide emulsion which has been exposed in the usual manner. The photographic element of the invention contains a sensitizing dye precursor. During development, the colorless dye precursor which is incorporated in the emulsion becomes oxidized to a sensitizing dye. This sensitizing dye, liberated at the site of development, becomes attached to a nearby silver halide grain and spectrally sensitizes it. If this development has been carried out in total darkness, the emulsion can then be uniformly exposed to light of a color which will not affect the unsensitized grains but will affect the sensitized grains, after which it is developed a second time to amplify the original image. In an alternative procedure, the first development can be carried out under yellow safelights so that as soon as the sensitizing dye is formed, the dye sensitizes neighboring grains which immediately undergo development to produce an amplified image.

In accordance with the present invention, we have provided a novel silver halide emulsion and photographic element which can be processed to different photographic speeds in a simple, quick and inexpensive manner. The processing enables the photographic element to be developed to a selected photographic speed by a choice of developing conditions.

The novel multiple-speed photographic emulsion comprises a photosensitive silver halide, a mordanting agent and a colorless dye precursor which is oxidizable by an oxidized photographic developing agent to form in situ a dye which spectrally sensitizes the silver halide to radiation of a region of the spectrum other than the sensitivity of the emulsion prior to oxidation of the dye precursor. For example, the photosensitive silver halide can have only native sensitivity (i.e., to ultraviolet and far blue light) and the sensitizing dye formed during development can sensitize the undeveloped silver halide to the green region of the visible spectrum. As another example, the silver halide can be sensitized to the red region of the visible spectrum and the sensitizing dye formed during development can sensitize the undeveloped silver halide to the green region of the visible spectrum. The photographic element of the invention comprises an emulsion of this type coated on a support.

The method of the invention in general comprises (a) imagewise-exposing the element to radiation of the electromagnetic spectrum to form a latent image in the radiation-struck areas, (b) developing the latent image in the dark, whereby the oxidation products of the photographic development convert the colorless dye precursor contained in the emulsion to a sensitizing dye which is adsorbed by the adjacent silver grains in an imagewise pattern, (c) exposing the photographic element to uniform illumination with light which will be absorbed by the silver halide spectrally sensitized with the sensitizing dye formed during development (the silver grains not so spectrally sensitized will not be affected by this illumination), and (d) redeveloping the grains exposed during (c) above to allow a secondary stage of photographic amplification to take place by converting the imagewise spectrally sensitized, silver halide grains to metallic silver.

In saying that we subject the photographic element to "uniform" illumination in exposing it for the second time, we use the term "uniform" to distinguish from imagewise

exposure and do not mean to exclude the possibility of using the well-known processing techniques of "burning in" or "dodging," by means of which areas of over- or under-exposure can be compensated for by giving a more intense or less intense second exposure to such areas.

Optionally, the first development may be carried out under uniform illumination with light of a color not absorbed by the spectrally unsensitized silver halide crystals, but which is absorbed by the spectrally sensitized silver halide crystals formed during development. The development reaction provides an imagewise pattern of spectral-sensitizing dye which is adsorbed by the adjacent silver halide grains, and said grains will immediately become developable as they are exposed during the development step.

Photographic elements prepared according to this invention can be processed by various methods including processing in alkaline solutions containing conventional developing agents such as hydroquinones, catechols, amino-phenols, 3-pyrazolidones, phenylenediamines, ascorbic acid derivative, hydroxylamines, hydrazines, reductones and the like; web processing such as described in Tregillus et al. U.S. Pat. 3,179,517; stabilization processing as described in Russell et al. "Stabilization Processing of Films and Papers," PSA Journal, vol. 16B, August 1950; mono-bath processing as described in Levy "Combined Development and Fixation of Photographic Images with Mono-baths," Phot. Sci. and Eng., vol. 2, No. 3, October 1958 and Barnes et al. U.S. Pat. 3,392,019. If desired, the photographic elements of this invention can be processed in hardening developers such as those described in Allen et al. U.S. Pat. 3,232,761; in roller transport processors such as those described in Russell et al. U.S. Pat. 3,025,779; or by surface application processing as described in Example 3 of Kitze U.S. Pat. 3,418,132.

Particularly good results are obtained when the emulsions of the photographic elements of this invention contain an incorporated ballasted developing agent such as the ballasted hydroquinones, e.g., t-butyl hydroquinone. The use of incorporated ballasted developing agents reduces the migration of the oxidized developing agent from the sites of exposure and development. This thereby reduces the formation of the sensitizing dye away from the sites of development and produces a sharper amplified image. For best results the emulsion should contain a quantity of ballasted developing agent at least sufficient to completely develop all the silver halide of the emulsion if it were completely fogged. The exposed element is then processed by being contacted with an alkaline solution similar to the usual developer solutions except that the solution does not contain a developing agent.

The colorless dye precursor component of the photographic element of this invention is a compound of the formula:.



and is present in an amount sufficient to yield upon oxidation by oxidized developer products in the time required for development of the element a sensitizing amount of a dye of the formula:



In the above Formulae I and II:

(a) each  $R_1$  represents an alkyl group (including substituted alkyl) having from 1 to 18 carbon atoms and 70 preferably a lower alkyl group having from 1 to 4 carbon atoms (e.g., methyl, ethyl, propyl, isopropyl, butyl, secondary-butyl, isobutyl, tert-butyl, pentyl, hexyl, octyl, decyl, dodecyl, octadecyl, and an aralkyl group preferably aryl lower alkyl containing from 1 to 4 carbon 75

atoms in the alkyl moiety (e.g., benzyl,  $\beta$ -phenylethyl,  $\omega$ -phenylbutyl, etc.), a sulfoalkyl group, preferably sulfo lower alkyl containing from 1 to 4 carbon atoms in the alkyl moiety (e.g., 2-sulfoethyl, 3-sulfopropyl, 3-sulfobutyl, 4-sulfobutyl, etc.), a carboxyalkyl group, preferably a carboxy lower alkyl containing from 1 to 4 carbon atoms in the alkyl moiety (e.g., 2-carboxyethyl, 3-carboxypropyl, 4-carboxybutyl, etc.), a sulfatoalkyl group, preferably a sulfato lower alkyl containing from 1 to 4 carbon atoms in the alkyl moiety (e.g., 2-sulfatoethyl, 3-sulfatopropyl, 4-sulfatobutyl, etc.), an alkoxyalkyl group, preferably lower alkoxy lower alkyl containing from 1 to 4 carbon atoms in both the alkoxy and alkyl moieties (e.g., 2-methoxyethyl, 3-methoxypropyl, 4-propoxybutyl, etc.), an acyloxyalkyl group, preferably acyloxy lower alkyl containing from 1 to 4 carbon atoms in the alkyl moiety (e.g., acetoxyethyl, propanoylethyl, butanoylethyl, benzoyloxyethyl, tolyloxypropyl, etc.), an alkoxy carbonylalkyl group, preferably lower alkoxy carbonyl lower alkyl containing 1 to 4 carbon atoms in both the alkoxy and alkyl moieties (e.g., 2-methoxycarbonylethyl, 4-ethoxycarbonylbutyl, 2-butoxycarbonylethyl, etc.), a dialkylaminoalkyl group, preferably di-lower alkylamino lower alkyl containing 1 to 4 carbon atoms in the alkyl moieties (e.g., dimethylaminoethyl, diethylaminopropyl, diethylaminobutyl, etc.), a cycloaminoalkyl group, preferably cycloamino lower alkyl containing 4 to 6 atoms in the cycloamino moiety and 1 to 4 atoms in the alkyl moiety (e.g., 1-pyrrolidinylethyl, 4-morpholinopropyl, 1-piperidinobutyl, 2-pyrrolin-1-ylmethyl, etc.), an alk-enyl group, preferably lower alk enyl containing 2 to 4 carbon atoms, (e.g., allyl, 1-propenyl, 1-but enyl, 2-but enyl, etc.), or an aryl group including substituted aryl (e.g., phenyl, naphthyl, tolyl, xylyl, halophenyl such as p-chlorophenyl, p-bromophenyl, 2,4-dichlorophenyl, alkoxyphenyl such as methoxyphenyl, etc.);

(b)  $R_2$  represents hydrogen, an alkyl group, preferably a lower alkyl group containing from 1 to 4 carbon atoms (e.g., methyl, ethyl, propyl, isopropyl, butyl, sec-butyl, isobutyl, tert-butyl, etc.) or an aryl group (e.g., phenyl, naphthyl, 4-tolyl, 2-tolyl, 2,4-dimethylphenyl, etc.);

(c) each X represents an acid anion (e.g., halide such as chloride, bromide or iodide, p-toluenesulfonate, thiocyanate, sulfamate, perchlorate, fluoborate, methylsulfonate, ethylsulfonate, fluorosulfonate, 2,4-dinitrobenzenesulfonate, etc.); and

(d) each  $Z_1$  represents the nonmetallic atoms necessary to complete a heterocyclic nucleus containing 5 to 6 atoms in the heterocyclic ring, which nucleus can contain a second hetero atom such as oxygen, nitrogen, selenium or sulfur such as a thiazole nucleus (including substituted and unsubstituted benzothiazole and naphthothiazole nuclei and the like), e.g., thiazole, 4-methylthiazole, 4-phenylthiazole, 4,5-diphenylthiazole, 4-(2-thienyl)thiazole, benzothiazole, 4-chlorobenzothiazole, 4-methylbenzothiazole, 4-methoxybenzothiazole, 4-ethoxybenzothiazole, 4-phenylbenzothiazole, 5-chlorobenzothiazole, 5-bromobenzothiazole, 5-methylbenzothiazole, 5-methoxybenzothiazole, 5-ethoxybenzothiazole, 5-phenylbenzothiazole, 6-chlorobenzothiazole, 6-bromobenzothiazole, 6-methylbenzothiazole, 6-ethoxybenzothiazole, 5-methoxynaphtha [2,3-d]-thiazole, naphtho[2,1-d]thiazole, naphtho[1,2-d]thiazole, etc.; an oxazole nucleus (including substituted and unsubstituted benzoxazole and naphthoxazole nuclei and the like), e.g., oxazole, 4-phenyloxazole, benzoxazole, 5-chlorobenzoxazole, 5-methylbenzoxazole, 5-bromobenzoxazole, 5-methoxybenzoxazole, 5-ethoxybenzoxazole, 5-phenylbenzoxazole, 5-methoxy-naphth[2,1-d]oxazole, etc.; a selenazole nucleus (including substituted and unsubstituted benzoselenazole and naphthoselenazole nuclei and the like), e.g., selenazole, 4-methylselenazole, 4-nitroselenazole, 4-phenylselenazole, benzoselenazole, 5-chlorobenzoselenazole,

6 - chlorobenzoselenazole, naphtho[2,1-d]selenazole, etc.; and a 2-quinoline nucleus (e.g., 2-quinoline, 5-ethyl-2-quinoline, 6 - chloro-2-quinoline, 8 - chloro-2-quinoline, 4-methoxy-2-quinoline, 8 - hydroxy-2-quinoline, etc.).

Typical dye precursors represented by Formula I above include:

- (A) 2,2'-trimethylenebis-(3 - ethylbenzothiazolium perchlorate);
- (B) 2,2'-trimethylenebis - (3 - methylbenzoxazolium iodide);
- (C) 2,2'-trimethylenebis-(3 - ethylbenzoselenium p-toluenesulfonate); and
- (D) 2,2'-trimethylenebis-(1 - methylquinoline perchlorate).

The novel photographic emulsions of this invention can be made by any of the well-known emulsion-making techniques in which the various components such as the vehicle, e.g., gelatin, the silver salt and other addenda are blended together. A suitable concentration of dye precursor is from 3 to 1000 mg. of dye precursor per mole of silver with the preferred range being from 50 to 400 mg. of dye precursor per mole of silver.

In preparing the photographic elements of the invention, the emulsions containing the dye precursor are coated on a support such as film, glass or paper in amounts of 50 to 500 mg. Ag/ft.<sup>2</sup> and preferably in amounts of 100 to 250 mg. Ag/ft.<sup>2</sup> of support.

The following examples provide further understanding of the invention:

#### EXAMPLE 1

To 100 ml. of 5% aqueous gelatin solution is added 40 grams of silver iodobromide emulsion containing 100 grams of gelatin (1.36 kg. of emulsion per mole of silver), 2 ml. of a 7½% saponin solution and 0.5 ml. of a 10% formaldehyde solution.

To 25 ml. samples of this mixture are added:

Sample 1. Control, no addenda.

Sample 2. 2.0 ml. of a methanolic solution containing in 30 ml., 20 mg. of the compound 2,2'-trimethylene-bis-(3-ethylbenzothiazolium perchlorate).



The above two emulsions are coated on polyethylene terephthalate support at .006" wet thickness and dried.

The dried coatings are exposed for 1/6 second at one millimeter slit width in a Bausch and Lomb spectrograph. The film is then processed for 2 minutes at 70° F. in the following developer solution:

190.0 ml. distilled water  
0.2 gram 1-phenyl-3-pyrazolidone  
0.2 gram N-methyl-p-aminophenol sulfate  
10.0 ml. of 2.5 N sodium hydroxide, with the following results:

#### Relative speeds

|                                       | No lights | Yellow lights |
|---------------------------------------|-----------|---------------|
| Sample 1 (control)                    | 40        | 40            |
| Sample 2 (incorporated dye precursor) | 160       | 320           |

In the dark, the incorporated quaternary salt favorably influences the developability of the latent image, but more significant is the speed gain realized by processing under lights which are filtered with a Kodak Wratten 16 yellow filter to remove the blue light.

This speed gain is realized along with considerable image spreading, presumably due to the mobility of the released sensitizing dye or of the oxidized developer.

#### EXAMPLE 2

In order to decrease the mobility of the imagewise-released sensitizing dye, a developing agent (t-butylhydroquinone) is incorporated in the photographic emulsion. Solutions used in this preparation and/or in preparing a control emulsion are as follows:

##### Solution (1):

To 100 ml. of a 5% gelatin solution is added 42 grams of a silver iodobromide emulsion (0.3 $\mu$  cubes, sulfur plus gold sensitized and containing 80 grams of gel and 2.16 kg. emulsion per mole of silver), 2 ml. of a 7½% saponin solution and 0.5 ml. of a 10% formaldehyde solution.

##### Solution (2):

A developer-gelatin mixture is prepared by dissolving 2 grams of t-butylhydroquinone in 18 ml. of methyl alcohol and pouring this solution, while stirring, into 80 ml. of a 10% aqueous gelatin solution.

##### Solution (3):

A solution of the 2,2'-trimethylenebis-(3-ethylbenzothiazolium perchlorate) is made by dissolving 0.1 gram of the material in 100 ml. of methyl alcohol. Two emulsion coatings are prepared as follows:

##### Coating A:

To 10 ml. of solution (1) is added 4.3 ml. of solution (2) and a 5% gelatin solution to make a total of 15 ml.

##### Coating B:

To 10 ml. of solution (1) is added 0.7 ml. of solution (3) and 4.3 ml. of solution (2).

Coatings with .004" wet thickness are made on subbed polyethylene terephthalate film support.

The dried coatings are exposed for 1/125 of a second with a one-millimeter slit width in a Bausch and Lomb spectrograph. These coatings are processed for 2 minutes in the following solution at 70° F.

|                        |      |       |
|------------------------|------|-------|
| Distilled water        | ml   | 200.0 |
| 2.5 N sodium hydroxide | ml   | 10.0  |
| Sodium sulfite         | gram | 1.0   |
| Potassium bromide      | gram | 0.5   |

The results are as follows:

|                                                      | Relative speeds |               |
|------------------------------------------------------|-----------------|---------------|
|                                                      | No lights       | Yellow lights |
| Coating A (incorporated developer only)              | 80              | 80            |
| Coating B (incorporated dye precursor and developer) | 80              | 320           |

The incorporation of the developing agent as described in this example decreases the image spreading.

#### EXAMPLE 3

This example illustrates a further procedure for confining the development-released products by adding an extremely fine-grain Lippman emulsion with a large surface area that is capable of more effectively mordanting the released sensitizing dye. This is accomplished as follows:

To 100 ml. of a 5% gelatin solution is added 21 grams of a silver bromoiodide emulsion (as described in Example 2) and 21 grams of a very fine-grain Lippman-type emulsion containing 60 grams of gelatin and 2.14 kg. of emulsion per mole of silver.

To 100 ml. of the above preparation is added 6.8 ml. of a 0.1% methanolic solution of 2,2'-trimethylenebis-(3-ethylbenzothiazolium perchlorate), 43.2 ml. of a developer solution containing 2 grams of t-butylhydroquinone, 18 ml. methyl alcohol and 80 ml. of 10% gelatin,

2.0 ml. of 7½% saponin solution and 0.5 ml. of 10% formaldehyde.

Coatings 0.004-inch wet thickness are made on subbed polyethylene terephthalate film support.

The dried coatings are exposed on a Bausch and Lomb spectrograph at  $\frac{1}{600}$  of a second at a slit width of 1.0 mm. and processed for 2 minutes in the developer described in Example 2 with the following results:

|                                                        | Relative speed |               |
|--------------------------------------------------------|----------------|---------------|
|                                                        | No lights      | Yellow lights |
| Emulsion with incorporated developer and dye precursor | 40             | 160           |

The above examples illustrate the ability of an oxidizable dye precursor, when incorporated in a silver halide photographic emulsion, to amplify the latent image thereby providing a photographic element of various sensitometric speeds.

The photographic layers used in the practice of this invention may be coated by various coating procedures including dip coating, air knife coating, curtain coating or extrusion coating using hoppers of the type described in Beguin U.S. Pat. 2,681,294. If desired, two or more layers may be coated simultaneously by the procedures described in Russell U.S. Pat. 2,761,791 and Wynn British Pat. 837,095. This invention also can be used for silver halide layers coated by vacuum evaporation as described in British Pat. 968,453 and LuValle et al. U.S. Pat. 3,219,451.

The photographic layers and other layers of a photographic element employed and described herein can be coated on a wide variety of supports. Typical supports include cellulose nitrate film, cellulose ester film, poly(vinyl acetal) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alpha-olefin polymer, particularly a polymer of an alpha olefin containing 2 to 10 carbon atoms such as polyethylene, polypropylene, ethylene, ethylenebutene copolymers and the like.

The silver halide emulsions used with this invention may be unwashed or washed to remove soluble salts. In the latter case, the soluble salts may be removed by chill-setting and leaching or the emulsion may be coagulation washed, e.g., by the procedures described in Hewitson et al. U.S. Pat. 2,618,556; Yutzy et al. U.S. Pat. 2,614,928; Yackel U.S. Pat. 2,565,418; Hart et al. U.S. Pat. 3,241,969 and Waller et al. U.S. Pat. 2,489,341.

The silver halide emulsions used in accordance with this invention can comprise, for example, silver chloride, silver bromide, silver bromoiodide, silver chlorobromide, silver chloroiodide, silver chlorobromide crystals or mixtures thereof. The emulsions may be coarse or fine grain emulsions prepared by any of the well-known techniques, e.g., single jet emulsions such as those described in Trivelli and Smith "The Photographic Journal," vol. LXXIX, May 1939, (pp. 330-338), double jet emulsions such as Lippmann emulsions, ammoniacal emulsions, thiocyanate or thioether ripened emulsions such as those described in Netz et al. U. S. Pat. 2,222,264; Illingsworth U.S. Pat. 3,320,069; and McBride U.S. Pat. 3,271,157. Surface image emulsions may be used or internal image emulsions may be used such as those described in Davey et al. U.S. Pat. 2,592,250; Porter et al. U.S. Pat. 3,206,313 and Bacon et al. U.S. Pat. 3,447,927. If desired, mixtures of surface and internal image emulsions may be used as described in Lucky et al. U.S. Pat. 2,996,382. The emulsions may be regular grain emulsions such as the type described in Klein and Moisar, *J. Phot. Sci.*, vol. 12, No.

5, September/October 1964, pp. 242-251. Negative type emulsions may be used or direct positive emulsions may be used such as those described in Leemakers U.S. Pat. 2,184,013; Kendall et al. U.S. Pat. 2,541,472; Berriman U.S. Pat. 3,367,778; Schouwenaars British Pat. 723,019; Illingsworth et al. French Pat. 1,520,821; Ives U.S. Pat. 2,563,785; Knott et al. U.S. Pat. 2,456,953 and Land U.S. Pat. 2,861,885.

The photographic and other hardenable layers used in the practice of this invention can be hardened by various organic or inorganic hardeners, alone or in combination, such as the aldehydes and blocked aldehydes, ketones, carboxylic and carbonic acid derivatives, sulfonate esters, sulfonyl halides and vinyl sulfonyl ethers, active halogen compounds epoxy compounds, aziridines, active olefins, isocyanates, carbamides, and polymeric hardeners such as oxidized polysaccharides like dialdehyde starch and oxyguargum and the like.

The photographic emulsions and elements described in the practice of this invention can contain various colloids alone or in combination as vehicles, binding agents and various layers. Suitable hydrophilic materials include both naturally-occurring substances such as proteins, for example, gelatin, gelatin derivatives, cellulose derivatives, polysaccharides such as dextran, gum arabic and the like; and synthetic polymeric substances such as water-soluble polyvinyl compounds like poly(vinylpyrrolidone), acrylamide polymers and the like.

The described photographic emulsion layers and other layers of a photographic element employed in the practice of this invention can also contain alone or in combination with hydrophilic, water-permeable colloids, other synthetic polymeric compounds such as dispersed vinyl compounds such as in latex form and particularly those which increase the dimensional stability of the photographic materials. Suitable synthetic polymers include those described, for example, in Nottorf U.S. Pat. 3,142,568 issued July 28, 1964; White U.S. Pat. 3,193,386 issued July 6, 1965; Houck et al. U.S. Pat. 3,062,674 issued Nov. 6, 1962; Houck et al. U.S. Pat. 3,220,844 issued Nov. 30, 1965; Ream et al. U.S. Pat. 3,287,289 issued Nov. 22, 1966 and Dykstra U.S. Pat. 3,411,911 issued Nov. 19, 1968; particularly effective are those water-insoluble polymers of alkyl acrylates and methacrylates, acrylic acid, sulfoalkyl acrylates or methacrylates, those which have cross-linking sites which facilitate hardening or curing and those having recurring sulfobetaine units as described in Dykstra Canadian Pat. 774,054.

The photographic elements used with this invention may contain antistatic or conducting layers, such layers may comprise soluble salts, e.g., chlorides, nitrates, etc., evaporated metal layers, ionic polymers such as those described in Minsk U.S. Pat. 2,861,056 and Sterman et al. U.S. Pat. 3,206,312 or insoluble inorganic salts such as those described in Trevo U.S. Pat. 3,428,451.

The photographic layers employed in the practice of this invention can contain plasticizers and lubricants such as polyalcohols, e.g., glycerin and diols of the type described in Milton et al. U.S. Pat. 2,960,404; fatty acids or esters such as those described in Robijns U.S. Pat. 2,588,765 and Duane U.S. Pat. 3,121,060 and silicone resins such as those described in Du Pont British Pat. 955,061.

The photographic layers employed in the practice of this invention may contain surfactants such as saponin; anionic compounds such as the alkyl aryl sulfonates described in Beldsiefen U.S. Pat. 2,600,831; amphoteric compounds such as those described in Ben-Ezra U.S. Pat. 3,133,816 and water-soluble adducts of glycidol and alkyl phenol such as those described in Olin Mathieson British Pat. 1,022,878.

The photographic elements employed in the practice of this invention may contain matting agents such as starch, titanium dioxide, zinc oxide, silica, polymeric beads including beads of the type described in Jolley et al. U.S. Pat. 2,992,101 and Lynn U.S. Pat. 2,701,245.

The photographic elements used in this invention may contain brightening agents including stilbenes, triazines, oxazoles and coumarin brightening agents. Water soluble brightening agents may be used such as those described in Albers et al., German Pat. 972,067 and McFall et al. U.S. Pat. 2,933,390 or dispersions of brighteners may be used such as those described in Jansen German Pat. 1,150,274, Oetiker et al. U.S. Pat. 3,406,070 and Heidke French Pat. 1,530,244.

Spectral sensitizing dyes can be used conveniently to confer additional sensitivity to the light-sensitive silver halide emulsion of the multilayer photographic elements of the invention. However, as we have indicated, any spectral sensitizing dye included with the colorless dye precursor must not sensitize in the area of the electromagnetic spectrum where the dye formed from the colorless dye precursor by oxidized developer absorbs radiation. For instance, additional spectral sensitization can be obtained by treating the emulsion with a solution of a sensitizing dye in an organic solvent or the dye may be added in the form of a dispersion as described in Owens et al. British Pat. 1,154,781. For optimum results, the dye may either be added to the emulsion as a final step or at some earlier stage.

Spectral sensitizers which can be used include the cyanines, merocyanines, complex (tri or tetrานuclear) merocyanines, complex (tri or tetrานuclear) cyanines, holopolar cyanines, styryls, hemicyanines (e.g. enamine hemicyanines), oxonols and hemioxonols.

Dyes of the cyanine classes may contain such basic nuclei as the thiazolines, oxazolines, pyrrolines, pyridines, oxazoles, thiazoles, selenazoles and imidazoles. Such nuclei may contain alkyl, alkylene, hydroxyalkyl, sulfoalkyl, carboxylalkyl, aminoalkyl and enamine groups and may be fused to carbocyclic or heterocyclic ring systems either unsubstituted or substituted with halogen, phenyl, alkyl, haloalkyl, cyano or alkoxy groups. The dyes may be symmetrical or unsymmetrical and may contain alkyl, phenyl, enamine or heterocyclic substituents on the methine or polymethine chain.

The merocyanine dyes may contain the basic nuclei mentioned above as well as acid nuclei such as thiohydantoins, rhodanines, oxazolidenediones, thiazolidenediones, barbituric acids, thiazolinones and malononitrile. These acid nuclei may be substituted with alkyl, alkylenes, phenyl, carboxyalkyl, sulfonalkyl, hydroxyalkyl, alkoxyalkyl, alkylamino groups or heterocyclic nuclei. Combinations of these dyes may be used, if desired. In addition, supersensitizing addenda which do not absorb visible light may be included, for instance, ascorbic acid derivatives, azaindenes, cadmium salts and organic sulfonic acids as described in McFall et al. U.S. Pat. 2,933,390 and Jones et al. U.S. Pat. 2,937,089.

The sensitizing dyes and other addenda used in the practice of this invention may be added from water solutions or suitable organic solvent solutions may be used. The compounds can be added using various procedures including those described in Collins et al. U.S. Pat. 2,912,343; McCrossen et al. U.S. Pat. 3,342,605; Audran U.S. Pat. 2,906,287 and Johnson et al. U.S. Pat. 3,425,825.

The invention has been described in detail with particular reference to preferred embodiments thereof, but it will be understood that variations and modifications can be effected within the spirit and scope of the invention.

We claim:

1. A photosensitive silver halide emulsion containing a colorless organic compound having the following formula:

10

which is oxidizable by an oxidized photographic developing agent to form in situ a sensitizing amount of a spectral-sensitizing dye having the formula:



wherein (a) each  $R_1$  represents an alkyl group having from 1 to 18 carbon atoms, a phenyl group, a substituted phenyl group, a naphthyl group, a substituted naphthyl group or an alkenyl group, (b)  $R_2$  represents hydrogen, a lower alkyl group, a phenyl group, a substituted phenyl group, a naphthyl group or a substituted naphthyl group, (c)  $X$  represents an acid anion and (d) each  $Z$ , represents the non-metallic atoms necessary to complete a heterocyclic nucleus containing 5 to 6 atoms in the heterocyclic ring, in the time required for development of the emulsion by said agent.

2. A photosensitive silver halide emulsion containing a colorless dye-precursor compound of the formula:



said compound being present in an amount sufficient to yield upon oxidation a spectrally sensitizing amount of a dye of the formula:



wherein (a) each  $R_1$  represents an alkyl group having 1 to 18 carbon atoms, a phenyl group, a substituted phenyl group, a naphthyl group, a substituted naphthyl group, or an alkenyl group, (b)  $R_2$  represents hydrogen, a lower alkyl group, a phenyl group, a substituted phenyl group, a naphthyl group or a substituted naphthyl (c)  $X$  represents an acid anion and (d) each  $Z_1$  represents the non-metallic atoms necessary to complete a heterocyclic nucleus containing 5 to 6 atoms in the heterocyclic ring.

3. An emulsion according to claim 2 wherein each  $Z_1$  represents the nonmetallic atoms necessary to complete a heterocyclic nucleus selected from the group consisting of a thiazole nucleus, an oxazole nucleus, a selenazole nucleus and a 2-quinoline nucleus.

4. An emulsion according to claim 2 in which said dye-precursor compound is 2,2'-trimethylenebis(3-ethylbenzothiazolium perchlorate).

5. An emulsion according to claim 2 which is free of sensitizing amounts of dyes that spectrally sensitize to the same wavelength as the dye to which said dye-precursor compound sensitizes when it is oxidized.

6. An emulsion according to claim 2 which also contains a mordant for the dye formed by oxidation of said dye-precursor compound.
7. An emulsion according to claim 6 in which said mordant is a fine-grain Lippmann emulsion which is admixed with the photosensitive silver halide emulsion in an amount sufficient to inhibit migration of the sensitizing dye formed from said dye-precursor compound.

8. A photographic element comprising a support and an emulsion according to claim 1.

9. A photographic element comprising a support and an emulsion according to claim 2.

10. A photographic element comprising a support and an emulsion according to claim 3.



**11**

11. A photographic element comprising a support and an emulsion according to claim 4.

12. A photographic element comprising a support and an emulsion according to claim 5.

13. A photographic element comprising a support and an emulsion according to claim 6.

14. A photographic element comprising a support and an emulsion according to claim 7.

15. A photosensitive silver halide emulsion containing 2,2'-trimethylenebis(3-ethylbenzothiazolium perchlorate) and t-butyl hydroquinone. 10

16. A photographic element comprising a support and an emulsion according to claim 15.

**12****References Cited****UNITED STATES PATENTS**

|             |        |                |        |
|-------------|--------|----------------|--------|
| 3,498,785   | 3/1970 | Bloom et al.   | 96—3   |
| 3,100,703   | 8/1963 | Sprague et al. | 96—33  |
| 5 2,104,064 | 1/1938 | Zeh            | 96—133 |

ROLAND E. MARTIN, JR, Primary Examiner

J. L. GOODROW, Assistant Examiner

U.S. CL. X.R.

96—54, 137